

84

Feb. 5, 1924.

1,482,480

H. W. MOWERY

LINING PLATE FOR BANK VAULTS AND SIMILAR STRUCTURES

Filed May 19, 1922

T19

H67  
H5



Harold Weaver Mowery  
INVENTOR

BY A. Parker Smith  
His ATTORNEY

Patented Feb. 5, 1924.

1,482,480

## UNITED STATES PATENT OFFICE.

HAROLD WEAVER MOWERY, OF MAHWAH, NEW JERSEY, ASSIGNOR TO AMERICAN  
ABRASIVE METALS COMPANY, A CORPORATION OF NEW YORK.

## LINING PLATE FOR BANK VAULTS AND SIMILAR STRUCTURES.

Application filed May 19, 1922. Serial No. 562,225.

*To all whom it may concern:*

Be it known that I, HAROLD WEAVER MOWERY, a citizen of the United States of America, residing at Mahwah, in the county of Bergen and State of New Jersey, have invented certain new and useful Improvements in Lining Plates for Bank Vaults and Similar Structures, of which the following is a specification.

10 My invention relates to linings or other portions of the walls of bank vaults, safes and other structures in which great powers of resistance to the attacks of thieves and burglars are required. In the modern art 15 of "safe-cracking" and bank robbing the use of electric drills, cutting torches and explosives has been brought to a high state of development and an equal degree of ingenuity is required to foil these attacks and protect the contents of the safes and vaults.

I have discovered that an important factor in the problem is the strength of the plate as a whole, as well as the high melting point and great hardness which give it its power 25 of resistance to drills and cutting torches. The particular function of strength is exerted in extending the effect of any explosions sufficiently to bring down a large quantity of débris consisting of large masses of 30 vault and building walls which may itself form a barrier to further progress insurmountable in the limited time available to the burglar. Such increased strength also tends to increase the noise of the explosion, which, of course, acts as an alarm.

To this end my invention relates more specifically to improving the character of the cast metal matrix in which masses of higher refractory character have heretofore 40 been embedded according to the previous patents to Ralph S. Edmondson, No. 1,423-652, granted July 25, 1922, and Francis J. Napolitan, Nos. 1,422,295, granted July 11, 1922, and 1,464,102, granted August 7, 1923. 45 My invention has also increased the resistance to drills and cutting torches of such plate matrices. It comprises the employment of a ferrochrome alloy for the matrix, in place of ordinary cast iron heretofore used.

I have discovered that such an alloy of 7% chromium and 93% iron gives the best results. A higher percentage of chromium increases the hardness, but decreases the

strength. While 7% of chromium gives the best results, variations between limits of from 5% to 10% of chromium content might be permissible in certain cases.

This alloy fulfills all the requirements which must be met to furnish a practical solution of the problem. It has great strength. A cylindrical test bar 1 $\frac{1}{4}$  inches in diameter placed on supports 12 inches apart will support a load of over 3500 lbs. applied midway between the supports. Its hardness is above that represented by "6" on the Brinnel hardness scale, which is far above the point now considered sufficient to render a substance practically drill-proof. It has a relatively high melting point and, if melted, solidifies at a slight reduction of temperature, so that it then forms masses which serve to partly clog up the hole the cutting torch is trying to bore. At the same time its melting point is not so high that it is impracticable to cast it, and the cost is not prohibitive.

This is the only material, out of many I have tested, which possesses all the conflicting qualities above described to a sufficiently high degree to satisfactorily resist drills, cutting torches and explosives.

The best form of structure at present known to me embodying my invention is illustrated in the accompanying figure of drawing which shows a cross-section of the preferred form of plate, and in which 1 represents the matrix or body of a plate formed of my ferro-chrome alloy, and 2, 2, represent irregular masses of still more refractory, but more brittle, metallic oxides embedded in the stronger matrix 1.

In some cases it might be possible to dispense with the masses 2, 2, and rely on the powers of resistance to drill and cutting torch of a solid plate made of the ferro-chrome alloy 1.

Having described my invention, I claim:

1. A plate for use in constructing the walls of bank vaults and similar structures composed of masses of refractory metallic oxides cast in a ferro-chrome matrix.

2. A plate for use in constructing the walls of bank vaults and similar structures composed of masses of refractory metallic oxides cast in a ferro-chrome matrix containing approximately 7% of chromium.

HAROLD WEAVER MOWERY.